

## UNITED STATES PATENT OFFICE

2,009,714

## FREE MACHINING CARBON STEEL

Frank R. Palmer, Reading, Pa., assignor to The Carpenter Steel Company, Reading, Pa., a corporation of New Jersey

No Drawing. Original application January 14, 1932, Serial No. 586,697. Divided and this application March 9, 1934, Serial No. 714,828

9 Claims. (Cl. 75—1)

This invention relates generally to ferrous products adapted for use in the manufacture of machined articles having relatively free machining quality imparted thereto by a selenium-tellurium content, as fully set forth in my copending application Ser. No. 586,697 filed January 14, 1932; the present improvement forming a division of the aforesaid application, and relating particularly to the so-called "straight carbon" class described therein.

In said application I pointed out that the ferrous alloys referred to might conveniently be divided into four general classes designated as "straight carbon" steels, "structural alloy" steels, "tool" steels and "special" alloy steels as fully described in said application. The invention described herein applies to the first of the before mentioned groups—namely, "straight carbon" steels, which is defined for my purpose as comprising all ferrous alloys containing more than 98% iron. The balance may consist of carbon, manganese and silicon with a small quantity of other alloying elements and a minimum of undesirable impurities, totalling not more than 2%. Providing the percentage of iron does not fall below 98%, ferrous alloys in this "straight carbon" group may contain small percentages of so-called alloying elements deliberately added but present in such small amounts as to hardly warrant their being called "alloy steels"; such elements as vanadium, tungsten, copper, molybdenum, chromium, nickel, sulphur, phosphorus, etc., being typical of the additions referred to. So-called "ingot iron", containing a minimum of non-ferrous elements, is also comprehended by the "straight carbon" group.

In the specifications of the American Society of Automotive Engineers, published in the S. A. E. handbook dated 1930 to which reference is made, the straight carbon steels are comprehended by the S. A. E. 1000 series. Obviously ferrous alloys can be compounded outside the limits of such S. A. E. specifications, as for example, copper bearing steels, or copper-molybdenum steels used for corrosion resistance, commercially pure ingot iron, tool steels containing more than 1.10% carbon, vanadium tool steels containing about .10% to .30% vanadium, etc., all of which for my purpose fall within the "straight carbon" group providing the iron content is more than 98%. Among the S. A. E. steels are found such compositions as X1315 containing low carbon, 1.25% to 1.55% manganese, .105% phosphorus, and .080% to .130% sulphur, which, since they contain more than

98% iron fall within the scope of my "straight carbon" steel group.

S. A. E. specifications provide for certain free machining types, as for example X1315, 1112 and 1120 which contain deliberately added sulphur with or without deliberately added phosphorus for purposes of free machining. Such high sulphur free machining steels have long been known but their commercial application is materially limited by the notoriously poor quality of the product. It is generally conceded that sulphur combines with some metal in the composition to form a metal-sulphide (usually manganese sulphide) having non-metallic slag-like properties. These inclusions are hardly soluble in the ferrous matrix,—having globular form in the cast ingot and being drawn out into long stringers in rolled or drawn products. In this form the inclusions greatly depreciate the transverse ductility of the metal and so decrease the general quality of the steel to a point which interferes with its commercial application,—notwithstanding the desirability of free machining properties.

I have determined that free machining properties may be introduced into these "straight carbon" steels by the addition of from .03% to 1.50% of the metalloids selenium and tellurium, used individually or jointly. Selenium and tellurium appear also to combine with a metal to form metal-selenides or metal-tellurides having non-metallic or slag-like properties. However, the selenides or tellurides appear to be largely soluble in the ferrous matrix because in any event they are found in much smaller quantities under the microscope than would be found with an equal percentage of sulphur in the composition. The smaller quantity of slag-like inclusions in the selenium or tellurium steels makes them much cleaner and more desirable for commercial applications; furthermore the transverse ductility is definitely higher than with equal percentages of sulphur due to the fact that continuity of the ferrous matrix is not interrupted to such a degree by slag-like stringers.

My experiments further indicate that selenium and tellurium are somewhat more potent than sulphur. For this reason when used in the same quantities as sulphur, the resulting machining properties are superior; or equal machining properties may be procured in my steel with smaller percentages of selenium or tellurium than would be required in a sulphur steel; which facts contribute further to the cleanliness and commercial applicability of my improved alloys. My experiments with tellurium confirm the

published medical statements regarding the poisonous nature of this element. Tellurium when added to a bath of molten steel gives off copious white fumes which are very disagreeable and dangerous to the workmen. Selenium also gives off white fumes, but these appear to be relatively unobjectionable as no poison effects have been observed by workmen even after several years experience with the use of selenium in the melting shop. I regard tellurium as particularly dangerous and objectionable in these "straight carbon" steels because such steels are usually made in open hearth furnaces and the metalloid additions would naturally be made in the ladle where there is little opportunity for the use of hoods or other safety devices for carrying off the tellurium fumes. For this reason I do not regard tellurium as practically available for my purpose although I have done enough work with it to determine that its presence in the steel achieves the purpose of my invention as was demonstrated for example by machining tests made on straight carbon steels of the following analysis:

25

| C   | Mn  | Si  | P    | S    | Te  |
|-----|-----|-----|------|------|-----|
| .15 | .73 | .23 | .008 | .030 | .15 |
| .06 | .35 | .85 | .014 | .029 | .34 |
| .05 | .22 | .04 | .008 | .028 | .40 |

In the case of selenium in which my work has been more extensive due to its non-poisonous nature I find that the machinability of straight carbon steels shows slight but noticeable improvement with percentages as low as .05% selenium and that the machinability increases progressively as the selenium content is increased up to about .25%. Further additions of selenium up to 1.50% give further progressive improvement but at a slower rate so that I contemplate that practically all free machining "straight carbon" steels can be satisfactorily made with between .05% and .25% selenium. However, it is to be understood that percentages between .25 and 1.50 achieve the purposes of my invention and are objectionable only because of the cost of the larger addition,—the higher percentage of loss in making these large additions,—and the general deterioration in the cleanliness of the alloy by increasing the amount of non-metallic matter.

Quite small percentages of selenium can also be used to supplement small percentages of sulphur, the effect on machinability apparently being cumulative. For example many specifications limit sulphur to less than .04% or .05%, but when supplemented by as little as .03% selenium, the total percentage of sulphur-selenium metalloid may be as much as .07 or .08 which is sufficient to react favorably on the machining properties of the alloy. Thus my invention is commercially usable with selenium even as low as .03%.

The use of phosphorus in straight carbon screw stock such as S. A. E. 1112 is recognized by the art. Phosphorus has an embrittling effect which is sometimes desirable in producing free machining properties.

In the use of my invention on steels that are soft, tough or "stringy" to machine, there are apparent advantages to employing phosphorus in conjunction with selenium to further improve the machinability. The embrittling effect of phosphorus is progressive and can be used up to .50% in extreme cases, however the more normal

range would be between .05% and .25%; and in steels when higher quality is required, phosphorus may be limited between .05% and .12%. It appears that a slight increase in phosphorus may be particularly desirable when the percentage of selenium is deliberately kept low in the interest of making cleaner steel. For example I have melted a straight carbon steel of the following analysis:

5

|            |       |      |    |
|------------|-------|------|----|
| Carbon     | ----- | .48  | 10 |
| Manganese  | ----- | 1.10 |    |
| Silicon    | ----- | .25  |    |
| Phosphorus | ----- | .05  |    |
| Sulphur    | ----- | .02  |    |
| Selenium   | ----- | .09  | 15 |

In this steel a slight increase of phosphorus was deliberately provided because the selenium was considerably below the optimum percentage for easiest machining and yet the steel was found to have excellent machining properties—particularly when subjected to the difficult operation of gun barrel drilling. The anti-friction, non-galling property which is characteristic of steels containing sulphur, selenium or tellurium was also notable in this steel. The above example illustrates the maximum amount of non-ferrous alloy permissible under my definition of "straight carbon" steel, the alloys in this case adding up to 1.99%.

25

My invention as applied to mild steel for screw machine purposes is well embodied in the following example:

|            |       |      |    |
|------------|-------|------|----|
| Carbon     | ----- | .15  | 35 |
| Manganese  | ----- | .75  |    |
| Silicon    | ----- | .12  |    |
| Phosphorus | ----- | .008 |    |
| Sulphur    | ----- | .030 |    |
| Selenium   | ----- | .10  | 40 |

Such steel machines as well, or slightly better, than S. A. E. 1120 with which it was compared, and promises greater utility because of its relative cleanliness and freedom from slag-like inclusions.

45

I have also made high carbon tool steels containing selenium and have found them to be free machining compared to similar steels without selenium, and without loss of their normal ability to harden and without apparent loss to their cutting quality as tools. Such high carbon tool steels are well known to the art containing from about .90% to about 1.50% carbon and at least 98% iron. An example of such free machining high carbon tool steel is given in the following analysis:

|            |       |      |    |
|------------|-------|------|----|
| Carbon     | ----- | 1.11 | 55 |
| Manganese  | ----- | .29  |    |
| Silicon    | ----- | .29  |    |
| Phosphorus | ----- | .013 |    |
| Sulphur    | ----- | .011 |    |
| Selenium   | ----- | .20  | 60 |

In the manufacture of my improved steel I have used elemental selenium both in powder and stick form, but I find it more desirable to first make an alloy of iron and selenium containing approximately 50% iron and 50% selenium, and to use this for additions to the molten bath. The iron-selenium alloy is heavy and is better assimilated by the steel with less loss by volatilization. In the manufacture of low and medium carbon "straight carbon" steels in an open hearth furnace, the selenium is best added in the ladle by introducing it into the flowing stream during tapping. The loss will depend upon the condition of the metal and may range from 50% upwards, 75

particularly when a content of more than .15% selenium is sought. In the manufacture of high carbon tool steel in the induction electric furnace the iron selenium alloy can best be added to the bath a few minutes before tapping. The losses may range from 10% for a .10% selenium addition, up to 30% for a .30% selenium addition. In the electric arc furnace the iron selenium alloy is best added at the time of tapping but the losses will be less than the open hearth additions because the condition of the metal is better.

10 I have tested the machinability of "straight carbon" steels as described above both in the cast and rolled condition and find that my invention applies equally well to castings and rolled, forged or drawn products.

Having clearly set forth my invention I claim:

15 1. A substantially "straight carbon" steel containing more than 98% iron, .03% to 1.50% metalloid of the group selenium-tellurium, .05% to .50% phosphorus and characterized by relatively free machining properties.

20 2. A substantially "straight carbon" steel as set forth containing more than 98% iron, .03% to 1.50% selenium and characterized by relatively free machining properties.

25 3. A substantially "straight carbon" steel as set forth containing more than 98% iron, .03% to 1.50% selenium, .05% to .50% phosphorus and

characterized by relatively free machining properties.

4. A substantially "straight carbon" steel as set forth, containing more than 98% iron, between .05% and .40% of selenium and characterized by relatively free machining properties.

5 5. A substantially "straight carbon" steel as set forth, containing more than 98% iron, between .05% and .40% of selenium, .05% to .25% phosphorus and characterized by relatively free machining properties.

10 6. A "straight carbon" tool steel containing more than 98% iron, carbon between .90% and 1.50%, selenium .05% to .30% and characterized by relatively free machining properties.

15 7. A "straight carbon" tool steel containing more than 98% iron, carbon between .90% and 1.50% selenium .05% to .30%, .05% to .12% phosphorus and characterized by relatively free machining properties.

20 8. A relatively free machining iron containing .03% to 1.50% selenium, balance substantially all iron.

25 9. A relatively free machining iron containing .03% to 1.50% selenium, .05% to .50% phosphorus and balance substantially all iron.

FRANK R. PALMER.